

## UNITED STATES PATENT OFFICE

2,319,662

## LUBRICATING OILS

Elmer W. Cook, New York, N. Y., and William D. Thomas, Jr., Stamford, Conn., assignors to American Cyanamid Company, New York, N. Y., a corporation of Maine

No Drawing. Application October 31, 1941,  
Serial No. 417,311

7 Claims. (Cl. 252—46)

This invention relates to lubricating oils, particularly those of the type known as crankcase oils. Although the lubricating oils of the present invention are highly desirable for use in crankcases of passenger automobiles they are especially valuable for heavy duty use in truck, bus, aeroplane, marine and Diesel engines which operate for long periods of time at high temperatures.

The principal objects of the invention are to provide a lubricating oil of the heavy duty type which possesses excellent detergent properties, is resistant to oxidation and sludge formation, is non-corrosive to alloy bearings and other metal parts under conditions of extreme service and which is free from film formation and ring sticking tendencies.

These objects, and others which will appear hereinafter, are accomplished by us by providing a hydrocarbon lubricating oil containing a class of compounds having detergent, and other desirable properties. These compounds are designated broadly as acyl phenol monosulfides having the general formula



and the metal salts thereof. In the formula R<sub>1</sub> and R<sub>2</sub> are alkyl radicals having 1-20 carbon atoms and R<sub>3</sub> and R<sub>4</sub> are members of the group consisting of alkyl, aryl, alkoxyalkyl, aroxyalkyl, aralkyl, alkaryl and cycloalkyl radicals.

When conventional lubricating oils are subjected to high operating temperatures for long periods of time, as in heavy duty service, they tend to decompose with the formation of complex and objectionable oxidation and decomposition products. Under the high temperature conditions obtaining in the engine these decomposition products polymerize to form lacquer-like deposits on or between the moving parts causing these parts to stick. Even larger quantities of polymerization products remain dispersed in the partly oxidized crankcase oil, and are rapidly precipitated and form a sludge when the engine cools or when fresh oil is added to the engine. These precipitated sludges become caked on heated metal surfaces and cut down the effective life of the engine.

A number of oil soluble detergents of the type of metal soaps, phenolates and alcoholates have

been proposed and used in crankcase oils to dissolve or disperse the sludge and prevent lacquer deposits and stuck piston rings. Unfortunately, however, the great majority of these substances increase the rate of oxidation in a manner somewhat analogous to the accelerating action of the various metallic soaps or "driers" on the oxidation of varnish films, and their presence results in an increased concentration of acidic oxidation products in the oil. Increased quantities of these acidic oxidation products in the oil create in turn an even more serious difficulty for they attack and corrode alloy bearings commonly employed in internal combustion engines. Alloys composed of copper-lead, silver-cadmium, nickel-cadmium, etc. are widely used and are subject to attack by the acidic oxidation products formed in the oil.

Certain anti-corrosion agents which have no detergent properties, such as triphenyl phosphite and sulfurized sperm oil, have been added to lubricating oils in order to counteract the corrosive effect of the oxidation products of the oil. Although the detergents which have been previously mentioned and the anti-corrosion agents perform their individual functions in lubricating oils the two separate chemicals do not cooperate to produce a satisfactory anti-corrosion and detergent action when used together. The function of a corrosion inhibitor is to cover the bearing surfaces and other corrodable parts of the engine with a passivating film that prevents corrosion of the metal by the organic acids and other corrosive products in the oil. A detergent, as its name implies, operates to remove adhering solids in the metal parts of the engine and thus produce a clean metal surface. Consequently mixtures of a detergent with a corrosion inhibitor have proven to be ineffective over any extensive period of time since the detergent action of the sludge inhibitor tends to remove the corrosion inhibitor from the metal surface thus rendering it ineffective for the purpose intended.

The acyl phenol monosulfides and metal salts thereof which we employ avoid the above described difficulties by possessing detergent, anti-sludging and corrosion inhibiting action in the single compound. The compounds are heat-stable and are not easily decomposed in the oil because of the high operating temperatures often encountered. They are also practically water-insoluble and are not extracted from the oil by contact with water. In addition to their detergent and dispersing properties they have oil-

ness properties and many of them also act to lower the pour point of the oil.

The acyl phenol monosulfides and their metal salts which we employ are so very effective that it is possible to improve lubricating oils to a great extent by the use of very small amounts of the compounds. In lubricating oils intended for ordinary service where high temperatures occur only occasionally, from 0.1-0.8% of the acyl phenol monosulfide or its salt is sufficient. In heavy duty service it is generally advisable to use a little more, as for example 0.5-3.0% in the oil.

The extremely high solubility of these compounds in hydrocarbon oils leads to another important advantage, namely, the ease with which these compounds are blended with lubricating oils. This step is further simplified by our practice of dissolving them in ordinary types of lubricating oils to the extent of 50-80% for storage and shipping purposes. For this reason it will be understood that the appended claims are intended to cover lubricating oil compositions of such high concentration unless otherwise limited.

The acyl phenol monosulfides which we employ to prepare the improved lubricating oils of our invention are made by reacting an alkyl substituted phenol monosulfide with an acyl halide in the presence of anhydrous aluminum chloride. Ordinarily we employ 2 moles of the acylating agent for each mole of the phenol monosulfide in order that each phenyl radical of the phenol monosulfide may be substituted with at least one acyl group. The reaction may be carried out in either one or two steps, i. e. the phenol monosulfide may be first reacted with the acyl halide followed by the addition of aluminum chloride and further reaction, or all of these reactants may be mixed together and the mixture heated. In either case heating is continued until the evolution of hydrogen chloride which is eliminated in the reaction has subsided. The product of this reaction is probably a complex aluminum salt of the acyl phenol monosulfide. This product is then decomposed by the addition of an excess of cold dilute hydrochloric acid. The acyl phenol monosulfide thus formed may be separated from the reaction mixture by extraction with a solvent followed by washing and evaporation of the solvent. Various metal salts of the acyl phenol monosulfide may be obtained by neutralization with an appropriate salt-forming base or by double decomposition with its sodium salt. The compounds thus prepared are straw-colored to dark reddish-brown liquids of varying viscosity and are found to be extremely soluble in gasoline and lubricating oils.

The alkyl substituted phenol monosulfides which we employ in the above reaction are well-known products having the general structural formula:



in which  $R_1$  and  $R_2$  are alkyl groups of 1-20 carbon atoms and in which the OH group may occupy a position either ortho or para to the sulfur linkage. The alkyl groups  $R_1$  and  $R_2$  tend to promote solubility of the compounds in lubricating oils and in general the longer the chain the more soluble the compounds will be in oil.

The acyl halides which we employ may be of different kinds such as for example butyroyl

chloride, caproyl chloride, lauroyl chloride myristoyl chloride, stearoyl chloride, benzoyl chloride, amyl benzoyl chloride, amyl oxyacetyl chloride, naphthenoyl chloride, phenyl acetyl chloride, phenoxy acetyl chloride, phenyl stearoyl chloride and many others. The naphthenoyl chloride mentioned above is composed of a mixture of various cycloaliphatic acyl halides such as are prepared from naphthenic acids, a product of the petroleum industry.

The metal radicals which we introduce into the acyl phenol monosulfide molecule to form salts thereof include those metal salt-forming radicals such as aluminum, lead, zinc, magnesium, calcium, barium, strontium, etc. The metal salts may be prepared by simply neutralizing the acyl phenol monosulfide with an appropriate metal oxide or hydroxide or by methods of double decomposition, as illustrated in the specific example. We prefer to employ the alkaline earth metal salts of these compounds in our improved lubricating oil compositions.

The preparation of a number of these acyl phenol monosulfides and salts thereof will now be described in detail in the following examples. It should be understood, however, that this description is given merely for purposes of illustration and our invention is not to be limited to the particular compounds or the particular method of preparation described since other acyl phenol monosulfides may be employed without departing from the scope of the invention as set forth in the appended claims.

#### EXAMPLE 1

##### 2-stearoyl-4-amyl phenol monosulfide



92 parts by weight of 4-amyl phenol monosulfide was dissolved in 70 parts of A. S. T. M. and 153 parts of stearoyl chloride added with stirring. The mixture was then heated under a reflux condenser with stirring for 30 minutes after which time the evolution of hydrogen chloride had subsided. After cooling, 23 parts of anhydrous aluminum chloride was added and the resulting mixture heated to refluxing temperatures with stirring. Refluxing and stirring were continued for 2 hours, at the end of which time very little hydrogen chloride was being evolved. The reaction mixture was then cooled and 200 parts of cold dilute hydrochloric acid added. The mixture was stirred thoroughly and 150 parts by weight of toluene added. The aqueous layer was then separated and the solvent layer washed once with warm, dilute hydrochloric acid and twice with hot water. The solvent was then evaporated and 2-stearoyl-4-amyl phenol monosulfide recovered as a reddish-brown liquid, readily soluble in gasoline and lubricating oil, but practically insoluble in water.

#### EXAMPLE 2

The barium salt of 2-stearoyl-4-amyl phenol monosulfide was prepared by dissolving 50 parts of the compound prepared in Example 1 in a solvent made up of 30 parts of ethanol and 60 parts of toluene. 9.5 parts by weight of barium hydrate was then added to the solution and the mixture heated at 80-120° C. with stirring until

the barium hydrate had reacted and the water of neutralization had been expelled. Toluene was added from time to time to replace the solvent evaporated. After cooling, the solution was filtered from traces of inorganic barium salts and the solvent removed by evaporation. The barium salt thus obtained was an extremely viscous reddish-brown liquid believed to have the following formula:



Because of the high viscosity of this product, it is preferable to add a quantity of light lubricating oil before the solvent is completely evaporated. By doing this a 50% solution of the barium salt of 2-stearoyl-4-amylophenol monosulfide in lubricating oil is obtained which is much more convenient for handling and blending.

#### EXAMPLE 3

The heavy metal salts of 2-stearoyl-4-amylophenol monosulfide, such as those of tin and zinc, may be conveniently prepared by double decomposition in an ethanol-toluene solution, between the sodium salt of 2-stearoyl-4-amylophenol monosulfide and the appropriate metallic inorganic salt.

For example, 30 parts of 2-stearoyl-4-amylophenol monosulfide was dissolved in a mixture of 30 parts of ethanol and 10 parts of toluene. 27 parts of a sodium ethylate solution, prepared by dissolving 23 parts of metallic sodium in 377 parts of ethanol, was heated and the mixture warmed up to 75° C. until homogeneous. The temperature was then dropped to about 50° C. and 6.4 parts of stannous chloride, dissolved in 20 parts of ethanol, was gradually added with stirring. The mixture was then heated to 75° C. and 40 parts of toluene added. After cooling, the solution was filtered from sodium chloride and the filtrate evaporated. The stannous salt of 2-stearoyl-4-amylophenol monosulfide remained as a viscous, reddish-brown product.

#### EXAMPLE 4

The aluminum salt of 2-stearoyl-4-amylophenol monosulfide was prepared by dissolving 20 parts of the product prepared in Example 1 in 40 parts of toluene followed by the addition of 5½ parts of aluminum butylate. The mixture was stirred and heated at 110° C. for 30 minutes. The solvent was then evaporated, the last traces under reduced pressure, and the aluminum salt of 2-stearoyl-4-amylophenol monosulfide recovered as a viscous, reddish-brown liquid.

#### EXAMPLE 5

##### 2-lauroyl-4-amylophenol monosulfide



This compound was prepared by condensing 2 moles of lauroyl chloride with 1 mole of 4-amylophenol monosulfide.

phenol monosulfide in the presence of 0.70 mole of anhydrous aluminum chloride following the procedure described in detail in Example 1. The product was a yellow colored liquid insoluble in water but easily soluble in gasoline and lubricating oils.

The various metallic salts of this compound were prepared in the same manner described in Examples 2 to 4.

10

#### EXAMPLE 6

##### 2-butyryl-4-amylophenol monosulfide

15



20

This product was prepared by condensing 2 moles of butyryl chloride with 1 mole of 4-amylophenol monosulfide in the presence of 0.70 mole of anhydrous aluminum chloride. The product was a straw colored liquid insoluble in water but easily soluble in gasoline and lubricating oil. The various metal salts are prepared as previously described.

30

#### EXAMPLE 7

##### 2-stearoyl-4-methylphenol monosulfide

35



40

This compound was prepared by condensing 2 moles of stearoyl chloride with 1 mole of 4-methylphenol monosulfide in the presence of 0.70 mole of anhydrous aluminum chloride by the procedure described in detail in Example 1. The product was a yellow liquid insoluble in water and readily soluble in gasoline and lubricating oil.

45

#### EXAMPLE 8

The barium salt of 2-stearoyl-4-methylphenol monosulfide was prepared by neutralizing 60 parts of the monosulfide dissolved in 30 parts of ethanol and 60 parts of toluene with 21 parts of barium hydrate. The solution was then filtered and the filtrate evaporated. The product was a very viscous brownish-red material. This product was blended with 50% of a 10-W grade of lubricating oil. This blend was liquid when warmed but on cooling and standing it set to a thin gel.

60

#### EXAMPLE 9

##### 6-stearoyl-2-amylophenol monosulfide

65



70

This compound was prepared by condensing 2 moles of stearoyl chloride and 1 mole of p-(2-amylophenol) monosulfide in the presence of 0.70 mole of anhydrous aluminum chloride. The product was a reddish-brown liquid insoluble in water but easily soluble in gasoline and lubricating oil.

75

## EXAMPLE 10

100 parts by weight of 6-stearoyl-2-amyl phenol monosulfide was dissolved in 70 parts of ethanol and 120 parts of toluene and neutralized with barium hydrate. The solution was then filtered and the solvent evaporated, leaving the barium salt of 6-stearoyl-2-amyl phenol monosulfide as a thick reddish-brown liquid.

## EXAMPLE 11

*2-naphthenoyl-4-amyl phenol monosulfide*

This compound was prepared by condensing 143 parts of naphthenoyl chloride with 100 parts of 4-amyl phenol monosulfide in 60 parts of naphtha in the presence of 26 parts of anhydrous aluminum chloride following the general procedure described in Example 1. The product was a brown liquid insoluble in water, but easily soluble in gasoline and lubricating oil.

The barium salt of this compound was prepared by reacting 12 parts of barium hydrate with 30 parts 2-naphthenoyl-4-amyl phenol monosulfide dissolved in an alcohol-toluene solution.

## EXAMPLE 12

*2-naphthenoyl-4-methyl phenol monosulfide*

This compound was prepared by condensing 104 parts of naphthenoyl chloride with 50 parts of p-cresol monosulfide dissolved in 50 parts of naphtha solution in the presence of 20 parts of anhydrous aluminum chloride. The product was a brown liquid practically insoluble in water but readily soluble in gasoline and lubricating oil.

The barium salt of this compound was prepared by heating 35 parts of 2-naphthenoyl-4-methyl phenol monosulfide, dissolved in 25 parts of ethanol and 50 parts of toluene, with 5 parts of barium hydrate. The product was a viscous, stiff, brown colored liquid which was blended with 50% of a light lubricating oil for ease of handling.

The effectiveness of the above-described compounds in preventing corrosion of bearings in lubricating oils, under conditions of severe service, is demonstrated by the following results obtained by subjecting a S. A. E. No. 10 solvent refined Mid-Continent oil to the Standard Catalytic Indiana test. Samples of the oil containing varying amounts (0.3-0.4%) of the acyl phenol monosulfide were compared with the oil containing no additive.

## TABLE I

*Catalytic Indiana test*  
*Mid-Continent solvent refined oil*  
*70 hours at 341° F.*  
*Copper-lead bearing*

| Additive                                         | Per cent additive | Bearing loss, mg. Cu-Pb |
|--------------------------------------------------|-------------------|-------------------------|
| Control, no additive                             |                   |                         |
| Barium 2-stearoyl-4-amyl phenol monosulfide      | 0.3               | 328                     |
| Aluminum 2-stearoyl-4-amyl phenol monosulfide    | 0.3               | 136                     |
| 2-lauroyl-4-amyl phenol monosulfide              | 0.4               | 189                     |
| Barium 2-naphthenoyl-4-methyl phenol monosulfide | 0.4               | 204                     |
| Barium 2-stearoyl-4-methyl phenol monosulfide    | 0.4               | 190                     |
| 6-stearoyl-2-amyl phenol monosulfide             | 0.4               | 88                      |
| Barium 6-stearoyl-2-amyl phenol monosulfide      | 0.4               | 211                     |
|                                                  |                   | 88                      |

A solvent refined Pennsylvania 10-W grade oil was also subjected to the Catalytic Indiana test with the following results:

## TABLE II

*Catalytic Indiana test*  
*Solvent refined Pennsylvania oil*

|    | Additive                                               | Percent additive | Bearing loss, mg. Cu-Pb |
|----|--------------------------------------------------------|------------------|-------------------------|
| 10 | Control<br>Barium 2-stearoyl-4-amyl phenol monosulfide | 0.3              | 201                     |
|    | 2-stearoyl-4-amyl phenol monosulfide                   | 0.3              | 19                      |
|    | 2-naphthenoyl-4-amyl phenol monosulfide                | 0.4              | 2                       |
|    | 2-butryyl-4-amyl phenol monosulfide                    | 0.4              | 83                      |
|    |                                                        |                  | 110                     |

15 In both tests the walls of the test tube containing the oils were clean indicating that the various acyl phenol monosulfides employed in the test possessed considerable detergent action.

What we claim is:

20 1. A lubricating oil composition containing a predominating amount of a mineral oil and a compound selected from the group consisting of acyl phenol monosulfides of the general formula



30 in which R<sub>1</sub> and R<sub>2</sub> are alkyl groups having 1 to 20 carbon atoms and R<sub>3</sub> and R<sub>4</sub> are members of the group consisting of alkyl, aryl, alkoxyalkyl, aroxyalkyl, aralkyl, alkaryl and cycloalkyl radicals and metal salts thereof.

35 2. A lubricating oil composition containing a predominating amount of a lubricating oil and 0.1-3% of a compound selected from the group consisting of acyl phenol monosulfides of the general formula



45 50 in which R<sub>1</sub> and R<sub>2</sub> are alkyl groups having 1 to 20 carbon atoms and R<sub>3</sub> and R<sub>4</sub> are members of the group consisting of alkyl, aryl, alkoxyalkyl, aroxyalkyl, aralkyl, alkaryl and cycloalkyl radicals and metal salts thereof.

55 3. A lubricating oil composition containing a predominating amount of a lubricating oil and 0.1-3% of a compound selected from the group consisting of acyl phenol monosulfides of the general formula



60 65 in which R<sub>1</sub> and R<sub>2</sub> are alkyl groups having 1 to 20 carbon atoms and R<sub>3</sub> and R<sub>4</sub> are members of the group consisting of alkyl, aryl, alkoxyalkyl, aroxyalkyl, aralkyl, alkaryl and cycloalkyl radicals and alkaline earth metal salts thereof.

70 75 4. A lubricating oil composition containing a predominating amount of a lubricating oil and a minor amount of a compound selected from the

group consisting of acyl phenol monosulfides of the general formula



in which  $R_1$  and  $R_2$  are alkyl groups having 1 to 20 carbon atoms and metal salts thereof.

5. A lubricating oil composition containing a predominating amount of a lubricating oil and a

minor amount of 2-stearoyl-4-aminophenol monosulfide.

6. A lubricating oil composition containing a predominating amount of a lubricating oil and a minor amount of the barium salt of 2-stearoyl-4-aminophenol monosulfide.

7. A lubricating oil composition containing a predominating amount of a lubricating oil and a minor amount of the barium salt of 2-lauroyl-4-aminophenol monosulfide.

ELMER W. COOK.

WILLIAM D. THOMAS, JR.